

March 4, 1941.

H. A. DREFFEIN

2,233,474

METHOD OF HEAT TREATING METAL

Filed June 3, 1938

5 Sheets-Sheet 1



March 4, 1941.

H. A. DREFFEIN

2,233,474

METHOD OF HEAT TREATING METAL

Filed June 3, 1938

5 Sheets-Sheet 2



March 4, 1941.

H. A. DREFFEIN

2,233,474

METHOD OF HEAT TREATING METAL

Filed June 3, 1938

5 Sheets-Sheet 3



Inventor  
Henry A. Dreffein  
By Sheridan, Davis & Clegg  
Atty.

March 4, 1941.

H. A. DREFFEIN

2,233,474

## METHOD OF HEAT TREATING METAL

Filed June 3, 1938

5 Sheets-Sheet 4



Inventor.  
Henry A. Dreffein  
By:

Sheridan, Davis & Clegg  
Attys.

March 4, 1941.

H. A. DREFFEIN

2,233,474

## METHOD OF HEAT TREATING METAL

Filed June 3, 1938

5 Sheets-Sheet 5



Henry A. Dreffein  
by Sheridan, Loring, Coghill  
Attys

## UNITED STATES PATENT OFFICE

2,233,474

## METHOD OF HEAT TREATING METAL

Henry A. Drefein, Chicago, Ill.

Application June 3, 1938, Serial No. 211,481

8 Claims. (Cl. 263—52)

This invention relates to improvements in methods of heat treating metal and has for an object annealing, normalizing, or malleablizing of metal in the form of cold rolled strip, sheets, or the like, and castings.

Heretofore, in the normalizing of cold rolled strip, for example, it has been the practice in one method to encase the coiled strip in a species of single or double walled retort and to apply heat either to the exterior of said retort or between the walls. This is expensive and requires considerable time. In another practice, electrical heating means has been utilized for direct heating. Also, endeavors have been made to utilize indirect heating means by burning gas in appropriately arranged tubes to render them radiant. In this last process the heat to which such tubes must necessarily be subjected to obtain the desired heating of the strip or sheets is destructive of the tubes.

In my process I first preheat the cold rolled strip as it is fed through a preheating chamber, after being uncoiled and flattened. It is next passed through a main heating chamber to which is supplied partially burned fuel gas mixture abnormally rich in gas content so as to create a rich reducing atmosphere to preclude oxidation or tarnishing of the strip, at the same time efficiently and rapidly bringing it to the desired temperature and maintaining it at that point for the period of time requisite to effect the desired normalizing. After that a partial cooling is effected during passage of the strip through a chamber for that purpose, such partial cooling being preferably effected by air moving through tubes, the air thus being at the same time preheated for subsequent use in combustion of the gases supplied to the main and other heating chambers and units. Thereafter the strip is fed through a succession of cellular subdivisions of the main cooling chamber in its passage through which the strip is subjected to decreasing temperatures. A reducing atmosphere is maintained in these cells by the delivery of condensed and purified partial gases of combustion. The strip, after reduction of its temperature to the point where it is not readily oxidized, is discharged from the apparatus.

Another object consists in the utilization of a generally similar process except as to temperature ranges, to sheets or other metal articles for annealing the same.

Another object consists in the utilization of a generally similar process for the malleablizing of castings.

These and other objects will be more fully explained and set forth in the following specification and illustrated in the accompanying drawings in which:

Fig. 1 is a vertical longitudinal section through a portion of my improved apparatus, taken along the line 1—1 of Fig. 2;

Fig. 1a is a similar section of the remainder taken along the line 1a—1a of Fig. 2a;

Fig. 2 is a horizontal section taken along the irregular line 2—2 of Fig. 1;

Fig. 2a is a similar section taken along the irregular line 2a—2a of Fig. 1a;

Fig. 3 is a vertical transverse section taken along the line 3—3 of Fig. 1;

Fig. 4 is a similar section taken along the line 4—4 of Fig. 1;

Fig. 5 is a fragmentary section of journal sealing means;

Fig. 6 is a horizontal section of a modified form of the apparatus;

Fig. 7 is a vertical longitudinal section of the structure illustrated in Fig. 6;

Fig. 8 is a vertical transverse section taken along the line 8—8 of Fig. 6;

Fig. 9 is a horizontal section through a modified form of apparatus particularly adapted for use in malleablizing castings or the like; and

Fig. 10 is a vertical section through the structure of Fig. 9.

My apparatus generally is constructed, in the usual manner, of refractory materials, properly reinforced and supported, such details forming no specific part of my invention other than as they enter into the general combination.

In the structure illustrated in Figs. 1 to 4, at the charging end, designated by numeral 10, is provided a pair of feeding rolls 11 extending across the charging opening and arranged to grip the end of a strip or a sheet positively to feed it into and through the apparatus, there being a series of transverse, spaced, intermediate rolls 12, rotated at such speed as to make the peripheral linear velocity identical with the feeding rate, so that the metal will not be marred or scratched. It will be understood that the cold rolled strip, if coiled, will be unrolled and flattened before delivery into the furnace. At the discharge end 13 is provided a similar pair of pinch rolls, as they are termed, designated by numeral 14. These also assist in effecting the movement of the metal by gripping it and drawing it through the furnace. All of the rolls, for convenience, are driven by a common drive chain 15 and sprockets 17, one of the latter being provided for each of the inter-

mediate and feeding rollers, as illustrated in Figs. 2 and 2a, for example. This chain 16 may be conveniently actuated by an electric motor and speed reducer F, diagrammatically illustrated, for example, in Fig. 2a.

At the charging end of the furnace is provided what I term a preheating chamber A. Extending from one end of that is the main heating chamber B, there being a bridge wall or partition 18 between the two chambers. At the opposite end of the main heating chamber is a partial cooling chamber C from which in turn extends the final or main cooling chamber generally indicated by D. A bridge wall 19 partially separates chambers B and C and a similar wall 20 is located at the juncture of chambers C and D.

At one side of the main heating chamber B is provided a combustion chamber E, a wall 22 being located between B and E. At the top, this wall 20 is provided with a plurality of discharge ports 23. The end walls of the combustion chamber extend outwardly from the body of the structure and in one of them is provided a burner generally indicated by numeral 25 arranged to discharge the fuel mixture longitudinally of the chamber E. A small gap 26 is provided in the wall 22 adjacent the burner 25, this construction being generally similar to the combustion chamber, etc., of my earlier Patent No. 1,938,814 of December 12, 1933, although it should be understood that the gap 26 may be eliminated if so desired. Gas is supplied to the burner 25 through the supply pipe 27 suitably controlled, and an air supply pipe 28 is also provided and equipped with suitable regulating means not illustrated, so that the mixture of fuel, such as gas and air, may be regulated to obtain the desired results.

At the forward end of the floor or hearth of chamber B is provided an outlet port 30 from which extends a flue or duct 31 (see Fig. 1). This in turn communicates with top and bottom longitudinal flues 32 and 33 in one side wall of the preheating chamber A, suitable vertical ducts being provided to connect the flues 32 and 33 (see Fig. 1, for example).

Extending across between the side walls of chamber A, near the top and bottom thereof, and suitably spaced, are what I term radiant tubes 35. One end of each of these tubes terminates in communication with a flue 32 or 33 to receive a supply of fuel gas, while the other end projects beyond the opposite side wall of the chamber A and is upwardly turned at 35a for discharge of gases of combustion, as illustrated in Fig. 3. Associated with each of these is a plug or other suitable type of valve 37, shown as frusto-conical in form. I have illustrated the valves for each pair of corresponding top and bottom tubes 35 inter-connected through levers 38 and connecting rod 39, these mechanisms being provided in the form shown, with an operating handle 40 so that the valves may be simultaneously regulated for control of the pressure and flow in each pair of tubes simultaneously. At the opposite end of each tube is provided a pipe 42 extending through the adjacent side wall of the chamber A and connected through a branch 42a with an air supply pipe 43, and through another branch 42b with an auxiliary gas supply pipe 44. Suitable valves are provided in each of these branches for controlling air or gas or both when thereby supplied to the tubes 35.

Extending across the chamber C, near the top thereof, is a plurality of air pipes 45, each of which communicates at one end with a manifold

46 and at the other end with a delivery pipe 47 which is connected to the air supply pipe 28. The manifold 46 is connected through pipe 50 with a motor driven blower generally indicated by numeral 51.

Also leading from the interior of chamber C is an exhaust pipe 53 communicating with a cooler or condenser 54. This, in turn, is connected through the pipe 55 with a purifier 56, the primary purpose of which is to desulphurize gases 10 passing therethrough. This latter element may be of any suitable type such as is now used by gas manufacturers and others which employs iron oxide to desulphurize gases. Communicating with the purifier 56 through the pipe 58 is an ex- 15 hauster 59 operable to withdraw gases from the chamber C through the condenser 54 and purifier 56. Such gases are then delivered through the pipe 61 to a manifold 62, from which valve controlled branches 63 lead to the interior of the 20 chamber D. An extension 64 leads from said manifold to the interior of chamber A, there being a suitable valve 64a interposed in the line.

The main cooling chamber D is divided into a plurality of cells by means of swinging flaps or 25 gates 66 depending from the top of the chamber above each of the intermediate rolls 12. Coacting with these suspending flaps 66 are pivoted upwardly inclined aprons 67 arranged to lie loosely against the surface of each of the rolls 12 and in 30 conjunction with the corresponding vertical flap to form a cellular subdivision of the chamber, flap 66 being pivoted to lie loosely against or close to the upper surface of the rolls 12 so as to permit the passage of a sheet or strip without obstruc- 35 tion.

One of the branch pipes 63 communicates with each of the cells, as illustrated in Fig. 1a.

Extending across the cells thus formed, near the top and bottom thereof, are transverse water 40 tubes through which water is circulated to assist in cooling the strip or sheets passing therethrough. It is desirable to obviate as far as possible the escape of gases from the apparatus, and, conversely, to prevent the entrance of air 45 from the outside, and with that end in view I construct my rollers with tapered ends 12a from which project shaft portions 12b, the refractory lining and walls of the apparatus being apertured to conform to and closely surround the 50 ends of the rollers while permitting protrusion of the shaft portions which are mounted in suitable bearings, generally indicated by numerals 70. It is desirable to provide side plates 72 on the outside of the furnace walls and it is necessary to aperture these to accommodate the extended shaft portions 12b of the rollers. These apertures 72a in my construction are made larger than the shaft portions 12b to permit relative expansion or movement without binding 60 upon or cutting the shaft portions. To prevent the escape of gases or the entrance of air through these apertures 72a, I provide glands, generally indicated by numerals 73 and of conventional construction, around which are mounted short 65 tubular members 75 of flexible tubing, such members at their other end being seated upon bosses 72b projecting from side plates 72. These flexible tubes permit relative contraction and expansion of the rollers and side plate as well 70 as relative lateral movement thereof, at the same time substantially preventing the leakage of air or gas through the side walls.

Incidentally, I prefer to use well known alloy rollers resistant to high temperatures in the pre- 75

heating and main heating chambers, also in the partial cooling chamber, but in the main cooling chamber I use ordinary steel rollers centrally apertured for the passage of cooling water from a suitable source, not shown.

In normalizing cold roller strip, for example in the apparatus described above, fuel gas in admixture with air under pressure is delivered to the burner 25 and ignited and the relative proportions of air and gas are so adjusted that only partial combustion of the fuel gas results. I desire to maintain an abnormally rich mixture of partially burned gases in the main heating chamber to obviate the possibility of oxidation of the strip or other metal passing therethrough. I contemplate maintaining a gas mixture of in excess of fifteen per cent of unconsumed fuel gas and can increase the richness to a point where there is approximately fifty per cent of unconsumed gas in the mixture.

In order to utilize this unburned fuel gas, I deliver a substantial portion thereof through the port 30 and the associated ducts and flues. This rich mixture is then induced into and through the radiant tubes 35 by compressed air delivered through the pipes 42, the amount of such delivery being regulated by valves to complete the combustion of the unburned fuel mixture. Proper regulation of the valves 31 is made so as to control the heating effect as well as the flow and pressure of the gases through and in the tubes 35.

It is my desire to maintain a reducing atmosphere throughout the entire apparatus which entails the maintenance of a pressure upon the partially burned fuel gases at least equal to and preferably greater than the external atmospheric pressure. The operation of the burner is controlled to obtain such pressure which also requires a consideration of and overbalancing of the suction effect of the induction air from the pipes 42. In the event that additional fuel gas is required for the heating of and through the tubes 35, an auxiliary supply of gas may be obtained through the pipes 42b leading from the auxiliary gas supply 44 (see Fig. 3). It will be apparent that a portion of the partially burned fuel gases will flow beneath the bridge wall 18 into the chamber A if the pressure be properly regulated, and this will maintain the necessary pressure in such chamber, at the same time providing the desired reducing condition to prevent oxidation of the strip or sheets.

Purified and dehydrated gas may be admitted from pipe 64 in a desired amount into chamber A. I contemplate, when it seems desirable, to utilize this supply of cooled and purified gas to the preheating chamber A to oppose the entry thereto of the partially burned fuel gases directly from the main heating chamber beneath the bridge wall while at the same time maintaining a desirable reducing atmosphere of rich gas.

After the strip moves out of the chamber B into and through the chamber C, it is partially cooled by the cooling pipes 45 and at the same time serves to preheat the air passing through said pipes to the burner 25. I find it efficient and economical to use preheated air in some instances for combustion because it will increase the temperature of the resultant combustion and I may obtain the desired heating effect with less combustion than will otherwise be required, thereby enabling me to provide a richer mixture of partially burned gases to heat the strip, there-

by further reducing the probability of oxidation or tarnishing of such metal.

As the strip moves into the receiving end of chamber D, cooling thereof is continued, but by dividing the chamber into a number of cells, 5 as described, convection currents through the entire chamber are practically eliminated and each cell may be maintained at a marked lower temperature than its predecessor, so that cooling action is more rapid and more effective than 10 where a single cell or chamber is utilized. Also, by separate control of the cooling water and cooled purified gases delivered to each cell of the main cooling chamber, I am enabled to control the cooling rate of the metal passing there- 15 through, as will be apparent.

Also, the supply of the cooled purified gases is preferably controlled to set up pressure in the cells of the cooling chamber which will resist or prevent flow of the hot fuel gases beneath the 20 bridge wall from the main heating chamber while at the same time maintaining the desired reducing atmosphere of rich partially burned gas.

In normalizing strip with my apparatus I regulate the speed with which such strip is fed through the apparatus so that it attains a temperature of between 1300° F. and 1400° F. when it reaches the bridge wall 18. After movement into the main heating chamber B this temperature is quickly raised to around 1700° F. (preferably 1650° F. 30 to 1800° F.) and remains at about that point during the remainder of the travel through the chamber B, which therefore functions not only to bring the metal to the desired maximum temperature, but as a soaking chamber in which 35 such temperature is maintained until the proper action is had upon the metal. During the passage of the strip through the chamber C, cooling action is relatively slow and its temperature is brought to around 1400° F. at the time it reaches the bridge wall 20. In passing through the cellular chamber D the drop in temperature is more rapid and the strip is preferably brought to at least 200° F. at the point of discharge from said chamber. This I term for convenience a 45 non-oxidizing temperature because such strip is not susceptible to quick oxidation or tarnishing under normal conditions after that temperature is reached.

A generally similar process is practiced in the 50 normalizing of metal sheets other than cold rolled strip, it being apparent that if hot rolled sheets or the like are fed directly into the preheating chamber at high temperature, the radiant tubes will be called upon for a lesser heat contribution 55 than when the cold rolled strip is being heated, and, if desired, the preheating chamber may be utilized quickly to bring the hot sheets or metal closer to the desired maximum temperature before their movement into the main heating chamber and, likewise, the heat contribution from the combustion chamber associated with the main heating chamber will be correspondingly less, as will be apparent.

I may also utilize this apparatus for annealing strip or metal sheets, in which operation the metal is brought to a temperature of around 800° F. in passing through the chamber A and quickly raised to around 1350° F. after entrance into the chamber B, and maintained at that point 70 during the balance of their travel therethrough. Similarly, a partial cooling to approximately 1000° F. is obtained in the chamber C and this is brought more rapidly to 200° F. or less during passage through the main cooling chamber D. 75

In the process described I am able efficiently and economically to obtain the desired heat treatment of the strip or other metal by direct application of fuel gas mixture in a continuous operation and in such a manner as substantially to obviate the formation of scale upon or the oxidation of the metal, and at the same time contribute to the economy of operation by salvaging the unburned fuel for preheating use and for 10 the maintenance of a purified reduced atmosphere in the cooling chamber.

In Figs. 6 to 8 I have illustrated a slightly modified form of apparatus in which the intermediate supporting rollers have been eliminated 15 from the main heating and the partial cooling chambers. In lieu thereof I construct the bottom or hearth 100 of these chambers as a continuous tank in which is maintained a pool of molten lead 101 (during the operation of the 20 furnace) and the metal being treated is supported upon and moved over the surface of this molten pool. In this manner I am able to dispense with the use of expensive alloy rollers and to eliminate the objections of any rollers in 25 these zones of greater heat which are susceptible to the deposit of scale or growth which causes excrescences upon the surface of such rollers which has a tendency to scratch or mar the sheets supported and moving thereon. Various methods may be 30 employed to engage and initiate the said strip or sheets being treated. For example, an alloy sheet may be attached to each end of the strip and initially fed through the furnace, drawing after it the strip. At the conclusion of the 35 passage of the strip, the drive is continued until the alloy sheet at the rear end is moved completely into the furnace in engagement with each pair of pinch rolls ready for initiating the movement of another strip or sheet when so desired. 40 Other methods may be employed, as, for example, the use of a chain or tongs inserted through ports or the like at intervals along the side walls of the furnace.

In the form illustrated, in Figs. 6 to 8, ports 45 105 are provided in communication with the main duct 106 which in turn supplies the partially burned fuel gases through suitable flues or ducts through the charging ends of the radiant tubes, as in the form of Figs. 1 to 4.

50 A slightly modified form of roller drive is also provided comprising a motor and speed reducer unit diagrammatically illustrated in Fig. 6 and generally designated by numeral 110. A drive shaft 111 is driven by this last described mechanism and through suitable drive mechanism, including chains, sprockets and bevel gears, actuates the drive chains 112 at each end of the apparatus, the action and arrangement being otherwise generally similar to that illustrated 55 in Figs. 1 to 4, the modification being due to the elimination of the intermediate rollers and the main heating and partial cooling chambers.

In Figs. 9 and 10 I have illustrated a modified form of apparatus more particularly designed 60 for utilizing my process in the malleablizing of castings.

In this apparatus a charging vestibule 150 is provided at one end and a similar discharging vestibule 151 is located at the discharge end. 65 These are provided with suitable counter-balanced doors 152. A plurality of pairs of tracks 153 extend through and beyond the apparatus, being mounted upon suitable spaced partitions. The apparatus includes a preheating chamber H, a main heating chamber I, and a cooling

chamber J, bridge walls 154 defining these chambers, as illustrated in Fig. 10. A combustion chamber 160 is located at each side of the main heating chamber, the construction being otherwise generally similar to that illustrated in Figs. 5 1 to 4. It should also be noted that I find it desirable to reverse the structural arrangement of the combustion chambers and the associated burners etc., i. e. one burner is facing toward the discharge end of the furnace and the other 10 toward the charging end.

A counter-balanced sliding door 162 is located at each end of the structure, as illustrated in Fig. 10.

Extending transversely across the preheating 15 chamber, near the top and bottom thereof, are radiant heating tubes 165. The supporting abutments or walls for the tracks 153 are cut away or apertured at 166 to accommodate the lower radiant heating tubes, as illustrated in 20 Fig. 9. These tubes are supplied with partially burned fuel from the heating chamber and with compressed air for combustion, as in the structure illustrated in Figs. 1 to 4, and are similarly controlled. 25

Extending transversely across the cooling chamber J, near the top thereof, are spaced air pipes 167 which are in communication with a blower or the like and serve the dual purpose of cooling the material passing therebeneath and 30 of preheating the air used for cooling so that it may be utilized for admixture with the fuel gases delivered to the burners. Similar air tubes 168 extend across the cooling chamber J near the front end thereof, the track walls being 35 apertured or cut away at 169 to accommodate such tubes.

Also extending across the cooling chamber J, near the bottom thereof, are radiant heating tubes 170 similar in arrangement and operation 40 to the tubes 165, the track walls being apertured at 171 to accommodate them.

In the practice of my method as applied to malleablizing with the apparatus just described, a transverse row of cars charged with castings 45 is moved into the vestibule 150 and thereafter, the door 162 having been raised, these cars are moved into the preheating chamber H by a pusher indicated generally by numeral 172 and contact the trains already therein to move them a 50 step toward the discharge end. Simultaneously, the rear door 162 having been raised, a transverse row of cars and their contents will be discharged into the adjacent vestibule. In this manner a step by step movement through the 55 entire apparatus is imparted to the cars and their contents.

The radiant tubes are controlled so as to bring the castings in their travel through the chamber H to a temperature of approximately 1300° F. to 1400° F. and thereafter move into the heating chamber I where hot partially burned gases of combustion function to bring them to a desired maximum temperature around 1700° F. in a 60 short interval of time. This temperature is maintained for a soaking action during the remainder of travel of such castings through the chamber I.

After movement into the cooling chamber J 70 this temperature is dropped with relative quickness to approximately 1400° F. and is reduced more slowly during the balance of travel through this cooling chamber J until it is reduced to at least 800° F. at the point of discharge. This 75

final cooling may be checked if too rapid by use of some or all of the radiant tubes 169. As indicated, it is preferable to effect this final cooling at a relatively slow rate, as it is in the nature 5 of an annealing operation.

With the use of this apparatus I contemplate operation with a time cycle of from fourteen to fifty hours (depending upon the temperature control, character and size of castings etc.), as 10 contrasted with the time cycle of one hundred to two hundred hours now required in the intermittent or periodic pot type of treatment.

Sufficient pressure is maintained on the partially burned rich gases in the heating chamber 15 I to maintain the pressure throughout the entire apparatus at least as high as atmospheric, and preferably slightly above, to preclude entrance of outside air and there is sufficient flow in both directions from the heating chamber to 20 maintain a reducing atmosphere in all of the chambers, the same rich mixture described in my normalizing method being desirable in the malleabilizing process.

It will be apparent that the specific method 25 described hereinabove is susceptible of variation and modification, and I do not wish to be restricted to such disclosure except as the claims, properly interpreted in view of the prior art, must be so limited.

30 What I claim as new and desire to cover by Letters Patent is:

1. A process of treating material comprising subjecting such material to a thermal sequence including heating of such material in the heating zone directly by rich partially burned fuel gases, a portion of said partially burned gases being thereafter utilized for combustion in radiant tubes or the like for indirect heating of said material in another zone, and a portion of said partially 35 burned fuel gases from said heating zone being withdrawn and utilized to maintain a special atmosphere about said material in still another zone.

2. A process of treating material comprising 40 subjecting such material to a thermal sequence including heating of such material in the heating zone directly by rich partially burned fuel gases, a portion of said partially burned gases being thereafter utilized for combustion in radiant tubes or the like for indirect heating of said material in another zone, and a portion of said partially 45 burned fuel gases from said heating zone being withdrawn, subjected to additional treatment, and utilized to maintain a special atmosphere about said material in still another zone.

3. A process of treating material comprising 50 subjecting such material to a thermal sequence including heating of said material in a heating zone directly by rich partially burned fuel gases, a portion of said gases being thereafter utilized for combustion in radiant tubes or the like for indirect heating of said material in another zone, and a portion of said partially 55 burned fuel gases from said heating zone being cooled and utilized

for cooling said material in a cooling zone while maintaining a special atmosphere therein.

4. A process of treating material comprising subjecting such material to a thermal sequence including heating of said material in a heating zone directly by rich partially burned fuel gases, a portion of said gases being thereafter utilized for combustion in radiant tubes or the like for indirect heating of said material in another zone, and a portion of said partially 10 burned fuel gases being withdrawn from said heating zone, cooled, and dehydrated and subsequently utilized for cooling said material in a cooling zone while maintaining a special atmosphere therein.

5. A process of treating material comprising 15 subjecting such material to a thermal sequence including heating of said material in a heating zone directly by rich partially burned fuel gases, a portion of said gases being thereafter utilized for combustion in radiant tubes or the like for indirect heating of said material in another zone, and a portion of said partially 20 burned fuel gases from said heating zone being cooled and applied in subdivided amounts of differing temperatures to said material to progressively cool the same.

6. A process of treating material comprising 25 subjecting such material to a thermal sequence including heating of said material in a heating zone directly by rich partially burned fuel gases, a portion of said gases being thereafter utilized for combustion in radiant tubes or the like for indirect heating of said material in another zone, and a portion of said partially 30 burned fuel gases from said heating zone being cooled and delivered to a plurality of cellular chambers through which said material is passed to cool the same, the temperatures in said cellular chambers being successively and markedly lower in the direction of travel of said material.

7. A process of treating material comprising 35 subjecting such material to a thermal sequence including heating of said material in a heating zone directly by rich partially burned fuel gases, a portion of said gases being thereafter utilized 40 for combustion in radiant tubes or the like for indirect heating of said material in another zone, and air for admixture with and combustion of said fuel gases in said radiant tubes being pre-heated by passage through tubes or the like in 45 proximity to said material to simultaneously partially cool said material in its passage from the heating zone to a cooling zone.

8. A process of treating metal comprising 50 sequential treatment of such metal in a preheating zone, a heating zone, and a cooling zone, heating of said metal in said heating zone being effected directly by rich partially burned fuel gases, a portion of said gases being thereafter utilized for combustion in radiant tubes or the like in said 55 preheating zone for indirect heating of said metal, a portion of said gases being withdrawn from said heating zone, cooled, and delivered to said cooling zone to cool the metal passing therethrough by maintaining a reducing atmosphere.

60 HENRY A. DREFFEIN.

65